

# UNITED STATES PATENT OFFICE.

JESSE A. PATRICK, OF GEORGIANA, ALABAMA.

## CLEANING AND POLISHING COMPOSITION.

1,363,481.

Specification of Letters Patent. Patented Dec. 28, 1920.

No Drawing.

Application filed July 15, 1920. Serial No. 396,424.

To all whom it may concern:

Be it known that I, JESSE A. PATRICK, a citizen of the United States, and a resident of the town of Georgiana, county of Butler, State of Alabama, have invented certain new and useful Improvements in Cleaning and Polishing Compositions, of which this is a specification.

The object of my invention is to produce a novel and highly efficient cleaning and polishing composition for use in renewing the finish of automobile bodies, metal work, wood work, glass and other surfaces, which will function as a cleaner and at the same time act efficiently as a polish. The composition, made up in the proportions I have found by experiment to be correct, and which cannot be greatly varied without seriously impairing the action of the composition, works excellently on all of the surfaces mentioned and not only cleans but efficiently polishes and with very little work in the way of rubbing.

My composition is composed of the following, in the proportions named:

|                                                                                            |                     |
|--------------------------------------------------------------------------------------------|---------------------|
| Lubricating oil                                                                            | 16 parts            |
| Kerosene oil                                                                               | 8 parts             |
| Apple vinegar                                                                              | 4 parts             |
| Wood alcohol                                                                               | 4 parts             |
| Heavy black varnish—that known in the trade as "auto black" being the best for the purpose | $\frac{1}{2}$ part. |

The ingredients as set forth are essential; the heavy black varnish is necessary to avoid the effect of what is known as "smoke" or a filmy appearance of the cleaned surface. This "smoke" shows on cleaned surfaces if the composition is made up without the black varnish admixture. Made up as set forth the polish is lasting; affected very little by soap and water and highly satisfactory.

What I claim is:

A cleaning and polishing composition composed of substantially sixteen parts lubricating oil, eight parts kerosene oil, four parts apple vinegar, four parts wood alcohol, and one-fourth part heavy black varnish.

Witness my hand this July 13, 1920.

JESSE A. PATRICK.

Witnesses:

H. J. CRENSHAW,  
MARION RUSHTON,  
DANIEL W. TROY, JR.